

March 1, 1960

Z. V. MOUDRY

2,927,052

PROCESS OF PRODUCING OLIGODYNAMIC METAL BIOCIDES

Filed March 20, 1953



INVENTOR

ZDENEK V. MOUDRY,

BY *Stone, Boyden & Mack*  
ATTORNEYS.

1

2,927,052

**PROCESS OF PRODUCING OLIGODYNAMIC METAL BIOCIDES**

Zdenek Vaclav Moudry, Northfield, Ill., assignor to United States Movidyn Corporation, a corporation of Illinois

Application March 20, 1953, Serial No. 343,705

1 Claim. (Cl. 167—14)

This invention relates to an improved process for producing oligodynamic metal microbicides and to novel oligodynamic metal microbicides of increased efficiency. The present application is a continuation-in-part of my copending application, Serial Number 174,781, filed July 19, 1950, now abandoned.

In general, the invention relates to the production of oligodynamic metal microbicides by the reduction of oligodynamic metal salts, through the action of actinic light, in such a manner as to produce a stable dispersion of essentially nonagglomerated microparticles of the elemental metal. By microparticles, I refer to particles which do not exceed a few hundred angstrom units (A.U.) in mean dimension.

The term "oligodynamic metal" does not appear to have a clearly defined meaning in the art. In the specification and claim, I employ this term to define certain metals, namely, silver, copper, gold, antimony, arsenic, cadmium, cobalt, germanium, iridium, mercury, palladium, platinum, zinc, bismuth, rubidium, tellurium and thallium, which in microparticulate form have the power of producing oligodynamic death of microorganisms. Oligodynamic death, to be distinguished from "ordinary death" or "poisoning," refers to death brought about by an amount of the active material which is so small that ordinary death or poisoning could not account for the biological action.

A great amount of work has been done in the past to produce oligodynamic materials which would be commercially satisfactory, but very little in the way of satisfactory results appears to have been accomplished. Lack of success in this art prior to my invention appears to have resulted from inability to obtain adequately high biological activity, and from the difficulty in producing a satisfactorily stable dispersion of the particulate oligodynamic material. The present invention provides an improved process by which satisfactorily stable oligodynamic dispersions are produced which have many times the biological efficacy of oligodynamic materials heretofore produced. To my knowledge, the invention provides for the first time a particulate oligodynamic metal product wherein the mean dimension of the measurable particles is less than 200 A.U., and, according to one embodiment of my invention, I am able to produce a product wherein the mean size of the measurable particles is below 75 A.U. As will hereinafter appear, I ascribe to such extremely small particle size a major part of the responsibility for the increased efficacy of the products of my invention.

Products of my invention also possess a unique characteristic which I term "residual biological activity." I have found that when an oligodynamic dispersion prepared in accordance with the invention is brought into contact with a solid surface, such as a metal surface of a container or a piece of chemical apparatus or a fibrous web of paper or textile material, such surface is not only sterilized but also upon withdrawal of the solution and

2

subsequent contact of the surface with a heavily contaminated material, this latter material is sterilized by the biological action of oligodynamic material remaining upon the treated surface. I have observed that such residual biological activity persists through many weeks and through many contacts with contaminated liquids. While I can give no conclusive explanation for the existence of such residual activity, it appears that this phenomenon is dependent upon the existence in the oligodynamic product of extremely small particles, some of these particles being retained by a solid surface by reason of adsorption and mechanical trapping.

A further unique advantage of the invention lies in the production of oligodynamic particles each containing at least two metals in elemental but physically combined form. As will appear in detail hereinafter, the invention provides for the simultaneous reduction of a plurality of oligodynamic metal salts, or of one oligodynamic metal salt and the salt of a non-oligodynamic metal, in such manner that a material proportion of the metal micro-particles produced contain both metals in elemental form, the physical configuration and behavior of such composite particles conforming to the configuration and behavior of an alloy. I have observed that the use of a second metal salt, either oligodynamic or non-oligodynamic, results in production of microparticles of substantially smaller size and in a marked increase in the oligodynamic killing power of the product, which increase may be due wholly or in part to the smaller particle size.

The mode of action of oligodynamic metals upon microorganisms is imperfectly understood. For many years, it was thought that such action depended upon adsorption of the metal to the surface of the microorganism, but subsequent advances in colloid science and physical chemistry, and in methods and equipment for measuring quantitative chemical processes have led to rejection of this theory. It has also been suggested that the action is catalytic, that it depends upon the formation of metal peroxides, or upon existence of an alubuminoid, etc. None of these theories appear to be maintainable today, and it is now generally agreed that oligodynamic killing power varies inversely as the particle size or subdivision of the oligodynamic metal. This present theory can be substantiated by relating the oligodynamic activity to solubility, which in turn is related to particle size.

I have discovered that dispersions of oligodynamic metal microparticles smaller than 200 A.U. can be produced by preparing an aqueous solution of a water soluble salt of an oligodynamic metal containing a certain type of gelatin, and irradiating the solution with actinic light.

The particular gelatin employed is a critical feature of my invention, since the use of almost all types of commercially available gelatins is totally ineffective to produce stable dispersions of microparticles of oligodynamic metal of the median size above referred to. For my process to be operable to produce stable dispersions of such microparticles, the gelatin employed must have the characteristics of Knox Gelatin #841, manufactured by the Chas. B. Knox Gelatine Co., Knox Bldg., Johnstown, N.Y. Knox Gelatin #841 is a very clear, medium jelly strength, acid type gelatin made from fresh frozen pork skins by acid treatment and acid hydrolysis. This gelatin has a gel strength of 125-250, a viscosity of 20-40 millipoises in 6% aqueous solution at 60° C., and a pH of 3-5 in aqueous solution. This gelatin is very strongly positively charged in aqueous solution and has an isoelectric point of 7.8-8.3. The cation content is very low. Analysis of Knox Gelatin #841 shows an

ash analysis of .3%, substantially all of the ash being calcium, with very minute non-measurable traces of silicon, aluminum, iron and phosphates. The calcium constituent of the gelatin is present as calcium collagenates. It appears that the ash analysis of .3% is probably a practical minimum for the natural product, and that the calcium ash analysis can be increased to at least about 1.2%. This particular gelatin is manufactured from fresh-frozen pork skins by acid treatment and acid hydrolysis. During hydrolysis the characteristics above referred to change progressively and the desired gelatin is withdrawn as a fraction when these characteristics have reached their proper values.

The only known equivalent of Knox Gelatin #841 is the ordinary gelatin of commerce in Germany and Czechoslovakia. This gelatin is prepared from the skins of bovine animals, has a pH of 5.8 in water and, upon analysis, shows 2.67% ash consisting substantially entirely of calcium.

The gelatin functions as a protective colloid, isolating the oligodynamic metal particles as they are formed and thus substantially preventing agglomeration of the particles. Particle size of the product appears to be in part a function of the reaction rate, and perhaps of other reaction conditions, and I have found that reduction by actinic irradiation will readily produce measurable particle sizes on the order of 100 A.U. and smaller when the salt is reduced in the presence of a gelatin having the characteristics of Knox Gelatin #841, but that microparticles of this extremely small size cannot be prepared when other gelatins are employed.

The gelatin employed must be free from ionizable halogen, else the particle size of the oligodynamic metal will be inordinately large.

The relative proportions of water-soluble oligodynamic metal salt and gelatin may vary widely. Thus, on the basis of 100 cc. water, the oligodynamic metal salt may be present as .01-.90 parts by weight, and the gelatin as .01-.50 parts by weight.

The gelatin must be present in intimate association with the oligodynamic metal salt throughout the period of irradiation. Accordingly, I first prepare an aqueous solution of the salt and the gelatin, and then carry out irradiation.

For irradiation to be effective to produce the microparticulate product desired, I have discovered that the actinic light to which the solution is subjected must have an intensity of at least 45 milliwatts per square foot, that at least 40% of the total radiation must lie in the infrared portion of the spectrum, that at least 25% of the total radiation must lie in the ultraviolet portion of the spectrum, and that the ultraviolet portion of the radiation must include a material proportion of light emitted at 3130 A.U. and at 3660 A.U. If the intensity of the actinic light employed is materially less than 45 milliwatts per square foot, reduction will not proceed at a rate sufficient to give adequate elemental oligodynamic metal. As has been stated, it appears that the particle size of the product decreases as the rate of reduction increases, and it is accordingly desirable to maintain the irradiation at a high level of intensity so as to shorten the reaction time. It appears that the actinic light serves both to cause reduction and to break the reduced metal particles into particles of smaller size, and I have observed that if the intensity of the actinic light is materially below 45 milliwatts per square foot, the particle size of the product will be undesirably large. In general, the period of irradiation may be in the range of from a few seconds, when light of high intensity is employed, to about one hour when the intensity is decreased to about the minimum value just mentioned. It is desirable to make the intensity as high as possible, and I find that intensities on the order of 1000 milliwatts per square foot, attainable with presently available commercial ultraviolet lamps, are highly desirable.

In carrying out my process, I prefer to employ an apparatus of the type illustrated in Fig. 1. The initial solution of the oligodynamic metal salt, containing Knox Gelatin #841, is placed in the mixing and storage tank 1. This solution flows, at a rate determined by flow gage 2, into a trough 3, hence downwardly across the sloping irradiation surface 4 into the trough 5 and thence to the receiver 6. All parts in contact with the liquid material may be of stainless steel. Positioned above the irradiation surface 4 is a reflector 7 carrying dependent radiation shields 8. A series of ultraviolet lamps 9 is arranged in progression along the line of flow of the solution, the lamps being supported in any suitable manner below the reflector 7. The solution flows by gravity in a thin film over the surface 4 and is irradiated by actinic light from the lamps 9 until entering the trough 5. The time of irradiation may thus be adjusted by changing the angle of the irradiation surface 4, and the material may of course be run through the apparatus as many times as desired. In commercial practice, I prefer to make the irradiation time on the order of a few seconds, with only one pass of the solution through the apparatus. The thickness of the liquid film may be on the order of 1 mm. or less.

25 The following examples are illustrative:

*Example I*

|                                | Parts by wt. |
|--------------------------------|--------------|
| Distilled water                | 100          |
| Silver nitrate (reagent grade) | 5            |
| Knox Gelatin #841              | 2.3          |

The silver nitrate is dissolved in a portion of the water, a suspension of the gelatin in the remaining water is then prepared, and the silver nitrate solution and gelatin suspension combined. The resulting mixture is then passed through an irradiating device such as that shown in Fig. 1, the lamps being chosen to provide an actinic light of the spectral characteristics hereinbefore described and an intensity of about 1,062 milliwatts per square foot, and the apparatus being so constructed that the liquid suspension is subjected to such irradiation for approximately 15 seconds.

The resulting product is a stable aqueous dispersion of silver microparticles, the measurable portion of the particles having a median maximum dimension of 100 A.U.

This product was diluted with water to provide a dilution of 1:5,000,000 on a volume basis. For comparison, a control product was prepared by adding monomethyl-p-aminophenol sulphate as a reducing agent to an aqueous mixture of silver nitrate and gelatin, the median particle size of the resulting oligodynamic silver being approximately 400 A.U. The control product was diluted with water to a 1:5,000,000 dilution by volume. In each case, the water for dilution contained sufficient *Escherichia coli* to provide 50,000 organisms per cc. of final liquid. The two diluted solutions were allowed to stand for 24 hours and the number of living organisms was then determined by standard techniques as recommended by the Department of Agriculture. No viable organisms were found by repeated tests in the product of this example, while many viable organisms were found in the control product.

*Example II*

65 An aqueous suspension of silver nitrate was prepared in the same manner as explained in Example I, and the suspension was then passed through an irradiating apparatus of the type shown in Fig. 1, the irradiation period being 150 seconds, and the actinic light having the spectral characteristics hereinbefore described but an intensity of approximately 110 milliwatts per square foot. The resulting product was a stable aqueous dispersion of silver microparticles, the measurable portion of the particles having a median maximum dimension of 100 A.U.

This product was diluted to 1:5,000,000 as in Example I, the diluted product containing 50,000 *Escherichia coli* organisms per cc. of final liquid. The diluted product so obtained was compared with a control product identical with the control product of Example I. The two diluted solutions were allowed to stand for 24 hours and the number of living organisms was then determined. No viable organisms were found by repeated tests in the product of the present example, while many viable organisms were found still to be present in the control product.

*Example III*

An aqueous suspension of silver nitrate is prepared in the same manner as explained in Example I, and the suspension then passed through an apparatus of the type shown in Fig. 1, the irradiation period being one hour and the actinic light, having the spectral characteristics hereinbefore described, and an intensity of 45 milliwatts per square foot. The resulting product is a stable aqueous dispersion of silver microparticles, the measurable portion of the particles having a median maximum dimension less than 200 A.U.

The product was diluted to 1:5,000,000 as in Example I, the diluted product containing 50,000 *Escherichia coli* organisms per cc. of final liquid. After 24 hours, repeated tests showed no viable organisms present.

It will be noted that in the foregoing examples, the silver nitrate and Knox Gelatin #841 are present in a proportion of 5:2.3. On a purely empirical basis, this proportion is desirable from the standpoint of cost, flowability and oligodynamic metal content desirable for certain commercial purposes. The proportion of silver nitrate may be varied within the range of .01-90 parts by weight, and that of the gelatin within .01-50 parts by weight, based on 100 parts by weight water, without materially changing the particle size of the oligodynamic metal in the product.

While the examples are limited to silver nitrate for simplicity, the water soluble salt of any other oligodynamic metal, as herein defined, may be employed in the same proportion of .01-90 parts by weight.

Composite or plural metal microparticles having a median maximum dimension less than 200 A.U. can also be prepared in accordance with my invention. To accomplish this, I prepare an aqueous solution of a plurality of water-soluble metal salts, at least one salt being of an oligodynamic metal, the salts preferably having a common non-metallic ion. The non-metallic ion can in no case be sulphate or sulphite. If silver is one of the metals, the non-metallic ions must not be halogen. In this solution, I incorporate an ionizable-halogen-free gelatin having the characteristics of Knox Gelatin #841. I then irradiate the resulting suspension with actinic light of the spectral characteristics and intensity hereinbefore specified, for a period of from a few seconds to about one hour, in order to simultaneously reduce the plural metal salts.

The total combined quantity of the metal salts may be within the range of .01-90 parts by weight, based on 100 parts by weight of water. The gelatin may be present as .01-50 parts by weight on the same basis.

In addition to one salt of an oligodynamic metal, one or more salts of a non-oligodynamic metal having good alloy forming properties may be employed, such metals being aluminum, beryllium, cerium, chromium, iron, lead, lithium, magnesium, manganese, molybdenum, nickel, rhodium, silicon, strontium, tantalum, tin, titanium, tungsten, vanadium and zirconium.

When my invention is carried out in accordance with this embodiment, starting with at least two salts, the product contains a major proportion of microparticles each of which contain the metal of each salt in elemental but physically combined form. As is the case when only

one oligodynamic salt is employed, the microparticles of the product are substantially un-agglomerated, the dispersion is stable, and the measurable microparticles of oligodynamic metal range below 200 A.U. in the mean maximum dimension. However, I find that when at least two salts are simultaneously reduced by actinic light in accordance with the invention, the mean maximum dimension of the microparticles tends to decrease, and that products having a maximum measurable particle size of less than 75 A.U. are readily produced.

The precise mechanism of the plural salt reduction just referred to is not understood. It has been demonstrated that at least a material proportion of the particles produced are composite, and contain the metals of each salt in elemental but physically combined form. The physical behavior of the system is, in many respects, similar to that of a typical partially miscible solid system exhibiting a eutectic discontinuity. In an ideal case, and with one metal being present in a lesser proportion, the reaction in accordance with this embodiment of the invention, results in the complete disappearance, from the solution, of the metal present in the lowest concentration.

The following examples are illustrative of this embodiment of the invention:

*Example IV*

|                                | Parts by weight |
|--------------------------------|-----------------|
| Distilled water                | 100             |
| Silver nitrate (reagent grade) | 5               |
| Cupric nitrate (reagent grade) | 1.5             |
| Knox Gelatin #841              | 2.3             |

The two salts are dissolved in a portion of the water, a suspension of the gelatin is made in the remaining water, and the salt solution and gelatin suspension combined. The resulting mixture is then passed through an irradiating apparatus such as that shown in Fig. 1, the lamps being chosen to give an actinic light having the spectral characteristics hereinbefore specified and an intensity of about 1,062 milliwatts per square foot, the apparatus being so constructed that the liquid is subjected to such irradiation for approximately 15 seconds.

The product is an aqueous dispersion of oligodynamic metal microparticles, a major proportion of the microparticles containing both silver and copper in elemental but physically combined form, the mean longest dimension of the measurable microparticles being approximately 20 A.U., and the largest dimension of the preponderance of the measurable microparticles being in the range of 75 A.U. or less. The particles are essentially non-agglomerated and the dispersion is stable over long periods of time.

The product of Example IV was diluted to a concentration of 1:100,000,000 on a volume basis, the water for dilution including sufficient *Escherichia coli* to give 50,000 organisms per cc. of final liquid. A control product was prepared by reducing an aqueous solution of silver nitrate, containing gelatin, with monomethyl-p-aminophenol sulphate as a reducing agent, the resulting product having a particle size of about 400 A.U. The control product was diluted to a concentration of 1:100,000,000 in the same manner as the product of the present example, so that the diluted control product included the same concentration of *Escherichia coli*. Both products were allowed to stand for a period of 24 hours and were then tested for living organisms. Repeated tests showed no viable organisms in the product of the present example, while many viable organisms were found to exist in the control product.

*Example V*

An aqueous suspension of Knox Gelatin #841, silver nitrate and cupric nitrate, in the same proportions as in Example IV, was prepared and irradiated in the manner described. The intensity of the actinic light was 45 milli-

watts per square foot and the time of irradiation one hour.

The product is an aqueous dispersion of oligodynamic metal microparticles, a major proportion of the microparticles containing both silver and copper in elemental but physically combined form. The mean maximum dimension of the measurable particles is less than 200 A.U.

The oligodynamic killing power of the product of the present example was composed with that of a control product produced as described in Example IV, both products being diluted to a concentration of 1:100,000,000 containing 50,000 *Escherichia coli* per cc. of the final liquid. After 24 hours, no viable organisms could be detected in the product of this example, while many viable organisms were detected in the control product.

While silver nitrate and cupric nitrate were employed in these examples for purposes of simplicity, equivalent products can be prepared by using salts of a plurality of the other oligodynamic metals, as defined herein, or by using one oligodynamic metal salt and one or more salts of the non-oligodynamic metals hereinbefore recited.

As in the case of use of a single oligodynamic metal salt, this embodiment of the invention also requires the use of both a gelatin having the characteristics of Knox Gelatin #841 and actinic light of the intensity and spectral characteristics hereinbefore specified, if a stable dispersion of oligodynamic microparticles smaller than 200 A.U. is to be obtained.

Throughout the specification, I have referred to the size of the "measurable" portion of the oligodynamic particles. Particle size of the products of the invention has been determined with great care by the use of electronmicrographs wherein the particles were magnified on the order of 40,000 times, so that a particle of 1 mu appears in the photograph as a 4 cm. image. The average maximum dimensions of the greatest number of like particles was taken as the mean particle size. On this basis, the mean particle size of the measurable particles of the products of all of the examples herein is less than 200 A.U., and that of Example IV is 20-75 A.U. Proceeding in accordance with Example I, the mean particle size of the measurable particles of the product will always be less than about 100 A.U., the size diminishing as the intensity of irradiation is increased so that the reduction time is shortened. When plural salts are employed, the particle size will be smaller in each case than for the corresponding product produced from a single oligodynamic salt.

I have observed that, in addition to the measurable particles in the product, the electronmicrographs indicate the existence of extremely small, unmeasurable particles which are thought to be particles of the oligodynamic metal. With existing methods and equipment, it appears to be impossible to determine with any reasonable accuracy either the chemical nature or the effect of this "background material."

It will be noted that the invention produces stable dispersions of oligodynamic particles of extremely fine subdivision, and that the use of both the particular type of gelatin referred to and actinic light of the characteristics specified herein is necessary to obtain such a product. I have observed that, in addition to the question of particle size, stability is a most critical factor when dealing with oligodynamic materials. While it may be possible to produce oligodynamic products of fairly small particle size by the use of chemical reducing agents, I have found that products so produced are always characterized by lack of stability. Where a chemical reducing agent is employed, even in the presence of a gelatin having the characteristics of Knox Gelatin #841, the particles of oligodynamic metal in the product tend to agglomerate excessively, so that the effective particle size of the product increases with time.

Certain of the products of my invention, and particularly products prepared either from a silver salt alone

or from silver and copper salts, are non-toxic to humans even when consumed directly in highly concentrated form.

Oligodynamic products produced in accordance with my invention have wide commercial applicability. Aqueous dispersions of oligodynamic metal produced in accordance with the invention may be used directly to decontaminate or sterilize materials, structures and commodities of many types. Thus, food products, fruits, 10 vegetables, drinking water, and the like may be treated with the material by direct addition to destroy harmful living organisms initially present. The products of my invention may be employed to inhibit growth of algae and fungi in swimming pools and the like, to control slime 15 growth in paper mills, knitting emulsions and the like, and to control bacteria in secondary oil recovery processes.

Metal, plastic and fibrous structures of many types may be sterilized by applying thereto liquid dispersions prepared in accordance with the invention. Thus, the material may be employed to treat containers, pieces of 20 chemical equipment, surgical instruments, operating room equipment and the like. Fibrous structures such as surgical bandages, paper, wrapping materials, textiles, and 25 leather may be directly contacted with the products of the invention. In all such application, the oligodynamic products function initially to sterilize the structure, and the extremely small oligodynamic microparticles are adsorbed and mechanically trapped on the surfaces of 30 the structure to provide long lasting residual biological activity.

Because of the increased efficacy of my products and the effect of residual biological activity, they are particularly valuable for use as a counter-measure in biological warfare. Thus, food products and articles and utensils of every day necessity once contaminated may be treated with my products, as by a simple dipping operation, to initially sterilize the same and also to provide a lasting sterilizing effect.

I find that the products of the invention are effective as preservatives for such commodities as foods, furs, leather, paper, textiles and the like. They may also be used as general disinfectants, as topical remedies for athletes' foot and like afflictions, and as components for soaps, detergents, toothpastes, cosmetics, and the like.

It will be noted that a number of the foregoing applications are of primary importance because of the phenomenon, characteristic to my products, which I have referred to as residual biological activity. I have observed that this phenomenon occurs to a material extent 50 only when the particle size of the oligodynamic product is very small. Thus, the phenomenon is manifested by products containing oligodynamic metal particles smaller than 200 A.U., but apparently is not significantly manifested when the particle size is in the neighborhood of 400-1000 A.U. Further, it appears that the residual activity increases very greatly as the particle size is decreased below about 100 A.U., and is very marked when the particle size is in the range of 20-75 A.U.

This relation of residual activity to particle size is apparently explainable on two grounds. First, it appears that the smaller the particle size the greater is the amount of oligodynamic metal adsorbed and trapped on the treated surface. Second, it appears that the residual activity depends upon solubility of the oligodynamic metal adhered to the treated surface, so that the effect is negligible if the particle is inordinately large, even though the particle should be held on the treated surface.

I claim:

The process of producing oligodynamic metal microbicides comprising forming an aqueous solution of a water soluble oligodynamic metal salt containing a colloid stabilizing proportion of an ionizable-halogen-free 75 gelatin having a viscosity of 20-40 millipoises, an iso-

electric point of pH 7.8-8.3 and a pH of 3-5 and irradiating said solution for from several seconds to one hour with actinic light having an intensity of at least about 45 milliwatts per square foot, at least 40% of the total radiation lying in the infrared portion of the spectrum, at least 25% of the total radiation lying in the ultraviolet portion of the spectrum and a material portion of the radiation being emitted at 3130-3660 A.U., and thereby producing a stable colloidal dispersion of oligodynamic metal microparticles predominantly smaller than 200 A.U.

References Cited in the file of this patent

UNITED STATES PATENTS

- |           |          |                |
|-----------|----------|----------------|
| 1,685,204 | Schreier | Sept. 25, 1928 |
| 2,132,886 | Voelker  | Oct. 11, 1938  |
| 2,220,187 | Wilmans  | Nov. 5, 1940   |

FOREIGN PATENTS

- |        |        |                                            |
|--------|--------|--------------------------------------------|
| 53,404 | France | June 4, 1945                               |
| 41,770 | France | Jan. 16, 1933<br>(Addition to No. 656,569) |

OTHER REFERENCES

- F. E. Ross: The Physics of the Developed Photographic Image, D. Van Nostrand Co., New York, 1924, 10 p. 14.
- Baker: Photo. Emulsion Technique, 2nd ed., 1948, pp. 33-35.
- Yagi: Rev. Phys. Chem., Japan, vol. 14, pp. 115-127, 1940, through Chem. Abst., vol. 35, p. 4264.
- 15 Gutbier et al.: Kolloid-Z., vol. 30, 1922, pp. 31-35, through Chem. Abst., vol. 16, p. 1350.